

## UNITED STATES PATENT OFFICE

2,400,361

METHOD OF PRETREATING CELLULOSE TO  
FACILITATE ITS ACYLATION

Carl J. Malm and Loring W. Blanchard, Jr., Rochester, N. Y., assignors to Eastman Kodak Company, Rochester, N. Y., a corporation of New Jersey

No Drawing. Application August 4, 1942,  
Serial No. 453,566

3 Claims. (Cl. 260—229)

This invention relates to the manufacture of cellulose esters of fatty acids of 3-4 carbon atoms, in which a small amount of formic acid is employed in the pretreatment of the cellulose.

In the making of cellulose esters containing a substantial amount of acetyl, pretreatment of the cellulose with acetic acid is possible and, therefore, the cellulose is successfully activated without any serious problems arising. However, in the preparation of propionic or butyric acid esters of cellulose, containing little or no acetyl, the activation of the cellulose preliminary to its esterification, presents various problems. For instance, if acetic acid is employed for activating the cellulose, its removal is necessary before the esterification occurs. As propionic and butyric acids are not satisfactory by themselves for pretreating cellulose, it is necessary that some assistance be provided. U. S. Patent No. 2,113,301 discloses a method of activating cellulose, using propionic or butyric acid, in which water or alcohol is present in the pretreating acid, in order to sufficiently activate the cellulose so it can be esterified. This increases the amount of anhydride which is necessary and, therefore, increases the cost of the process.

An object of our invention is to provide a method of pretreating cellulose in which the only lower fatty acid groups present are substantially all propionyl or butyryl. Another object of our invention is to provide a method of making cellulose propionates and cellulose butyrates which is inexpensive but results in a product having good stability. Other objects will appear herein.

We have found that cellulose may be satisfactorily pretreated with propionic or butyric acid if but a small amount of formic acid is present in the pretreating liquid. We have found approximately  $\frac{1}{20}$  to  $\frac{1}{2}$  part of formic acid, per part of cellulose pretreated, gives good results, but not more than  $\frac{1}{2}$  part of formic acid is necessary or desirable in the operation.

Heretofore, formic acid has not been employed in esterification processes because in the usual types of esterification, i. e. acetylation, the formic acid has been dehydrated or decomposed by the acid anhydride used, either because of the high temperature of esterification or the large amount of catalyst employed, or both. Also, it has been thought that formyl groups combined with cellulose were very unstable and were readily broken off from the cellulose derivative in which they were found. We have found, however, that in the making of cellulose propionate or cellulose butyrate in which a liquid to cellulose ratio of not more than 7:1 is used, thereby making possible

the use of small proportions of catalyst, and the use of a weaker anhydride (such as butyric or propionic) in the esterification, that cellulose may be esterified in the presence of formic acid without decomposing any of the formic acid with the consequent waste of anhydride.

We have also found that the susceptibility of cellulose derivatives containing formyl groups, heretofore, toward instability, has been due to a 10 susceptibility towards hydrolysis resulting from the comparatively high water-susceptibility of the cellulose esters. We have found that in the case of cellulose propionates or cellulose butyrates in which only small amounts of formyl are present 15 that the products are not susceptible to water and, consequently, a stable product results.

The pretreatment method, as described in this application, is especially designed for use in combination with an esterification reaction in which 20 not more than seven parts of the liquid esterification mass is employed for one part of cellulose, and preferably the proportion is approximately 4.75 parts of liquid to 1 of cellulose. By thus maintaining a low liquid to cellulose ratio it is 25 possible to carry out the reaction at relatively low temperatures and with comparatively small amounts of catalysts. For instance, a satisfactory esterification, using propionic or butyric anhydride, can be carried out using a proportion of 30 sulfuric acid of 1-5% based on the cellulose and at an esterification temperature, the maximum of which is not more than 100° F. and preferably within the range of 70 to 90° F. Our invention is also especially adapted for the making of cellulose esters, substantially all of the acyl of which 35 consists of fatty acid radicals of 3-4 carbon atoms, the amount of acetic acid present in the esterification mass being no more than 5% and preferably none at all. As the liquid to cellulose ratio 40 is restricted, there would be substantially no solvent employed such as ethylene dichloride or chloroacetic acid, these being unnecessary in the esterification process.

It is preferred that the pretreatment of the 45 cellulose in accordance with our process be carried out by first treating a portion of the cellulose and after the treatment has occurred for a short time, the remainder of the cellulose is added and the mixing or stirring is continued until the 50 desired activation has occurred. Sulfuric acid is also employed in the pretreatment liquid and by adding the cellulose in a plurality of steps, ordinarily two, the initial cellulose added is partially broken down so that mixing, when the second or 55 subsequent portions of cellulose are added, goes more readily than where the cellulose is added

all in one portion. Although ordinarily the pretreatment is carried out at 100° F., other pretreatment temperatures may be employed. For instance, with lower temperatures such as down to 70° F., a slightly higher proportion of sulfuric acid is desirable in the pretreatment. Conversely, with a higher pretreatment temperature less sulfuric acid is used.

For the preparation of high viscosity esters it is also desirable to keep the proportion of sulfuric acid in the pretreating liquid relatively low. For example, it is ordinarily desirable to use approximately .001 part of sulfuric acid or less per part of cellulose to be esterified for preparing a high viscosity ester, if a pretreatment temperature of approximately 100° F. is to be used and a time of  $\frac{1}{4}$  to  $\frac{1}{2}$  hour is employed for the initial portion of the pretreatment. For lower viscosity esters, higher proportions of sulfuric acid may be employed in the pretreatment for the same temperature. If, however, the temperature is lower, higher proportions of sulfuric acid are permissible even for the higher viscosity esters, as pointed out above.

The pretreatment, in accordance with our invention, is ordinarily carried out in a mixer or other like vessel in which thorough mixing or kneading of the mass can be accomplished. The pretreating liquid, which is preferably less than two parts per part of cellulose to be activated, is placed in the mixer and the cellulose is added thereto, preferably, at first, a half portion of the cellulose to be activated. The mixing is carried out until the mass begins to mix more easily or until the cellulose exhibits physical break down or crumbliness. The remainder of the cellulose is then added and the mixing is continued until the cellulose is activated to the degree desired. Ordinarily the time for treatment of the first portion is  $\frac{1}{2}$  hour at 100° F., while after the addition of the second portion the mixing is continued for 1 hour at that temperature. However, the various conditions of operation, such as temperature, proportion of sulfuric acid, the type of cellulose being treated, etc., all exert an influence on the time necessary so that no hard and fast rule can be drawn as to the time of treatment necessary unless all the other conditions are also taken into consideration. Ordinarily the proportion of sulfuric acid which will be employed in the pretreatment, in accordance with my invention, will be from .00005 to .006 part per part of cellulose. A very satisfactory ratio of pretreating liquid to cellulose is approximately  $\frac{3}{4}:1$ . However, the proportion of liquid for pretreating the cellulose may be anywhere from  $\frac{1}{4}$  part to 2 parts per part of cellulose. With a small proportion of pretreating liquid it is sometimes desirable to add the cellulose in more than two portions in the pretreating operation. With a higher proportion of pretreating liquid, in some cases it may be desirable to initially add the cellulose as a whole. In those cases where a small proportion of pretreating liquid is employed, obviously a small proportion of formic acid is to be employed in the pretreating liquid, such as on the order of  $\frac{1}{8}$  part of formic acid per part of cellulose. The following examples illustrate our invention:

#### Example I

1½ pounds of cotton linters were added to a mixture of .6 pound of butyric acid, 90 cc. of 90% formic acid, and 1 cc. of sulfuric acid (sp. gr. 1.84) in a Werner-Pfleiderer type mixer and the

mass was mixed at 100° F. for  $\frac{1}{2}$  hour. A second portion of 1½ pounds of linters was then added and the mixing was continued for 1 hour at 100° F. 13 pounds of butyric anhydride were added, the mixture was cooled to 58° F. and a mixture of 20 cc. of sulfuric acid and 20 cc. of acetic acid were added. The reaction was allowed to proceed to a maximum temperature of 85° F. After 7½ hours a smooth, very viscous solution was obtained. A mixture of 2½ pounds of water and 10 pounds of butyric acid was then added and the mass was allowed to stand at 100° F. for sufficient time to hydrolyze the cellulose ester to the desired degree. The cellulose butyrate thus obtained was recovered by precipitation, washing, and drying. The resulting product was a cellulose butyrate containing about 1% combined formyl.

#### Example II

1½ pounds of cotton linters were added to a mixture of 1 pound of formic acid (90%),  $\frac{1}{2}$  pound of butyric acid, and 1 cc. of sulfuric acid in a Werner-Pfleiderer type mixer. The mixer was run for 1 hour at 100° F. and a further 1½ pound portion of cotton linters was added. The mixing was continued for 2 hours at 100° F. 13 pounds of butyric anhydride were added, the mixture was cooled to 55° F. and 20 cc. of sulfuric acid diluted with 20 cc. of acetic acid were then added. The reaction was allowed to proceed to a maximum temperature of 98° F. After 13 hours a smooth, homogeneous solution was obtained. The hydrolysis, precipitation, washing, and drying were carried out as in Example I.

The method which we have described is useful for the preparation of cellulose propionates, cellulose butyrates, or cellulose propionate butyrates, either fully esterified or hydrolyzed. The resulting products exhibited good stability as shown by the failure of the ester to develop any acidity upon boiling for 24 hours in distilled water.

We claim:

1. A method for activating cellulose to prepare it for esterification which comprises treating the cellulose with a mixture of a fatty acid of 3-4 carbon atoms, 0.3 to 0.5 part of formic acid per part of cellulose and a small proportion of sulfuric acid until the desired activation has occurred.

2. A process of preparing cellulose esters having a high content of fatty acid radicals of 3-4 carbon atoms which comprises mixing half the cellulose to be esterified with a pretreating liquid essentially consisting of fatty acid of 3-4 carbon atoms, 0.3 to 0.5 part of formic acid per part of cellulose and a small proportion of sulfuric acid at 100° F. for  $\frac{1}{2}$  hour, the proportion of pretreating liquid to cellulose to be esterified being approximately  $\frac{3}{4}:1$ , adding the remainder of the cellulose and continuing the treatment for one hour at 100° F. and subsequently inducing esterification by adding to the mass sulfuric acid and sufficient butyric anhydride to completely acylate the cellulose, the ratio of esterification liquid to cellulose being not allowed to exceed 7:1 and the esterification temperature not being allowed to exceed 100° F.

3. A method for activating cellulose to prepare it for esterification which comprises treating the cellulose with a mixture of a fatty acid of 3-4 carbon atoms, 0.3 part of formic acid per part of cellulose, and a small proportion of sulfuric acid until the desired activation has occurred.

CARL J. MALM.

LORING W. BLANCHARD, JR.